

# UNITED STATES PATENT OFFICE.

WILHELM ELBERS, OF HAGEN, GERMANY, ASSIGNOR TO THE BADISCHE ANILIN AND SODA FABRIK, OF LUDWIGSHAFEN, GERMANY.

## GRAY CLOTH AND PROCESS OF DYEING SAME.

SPECIFICATION forming part of Letters Patent No. 650,752, dated May 29, 1900.

Application filed June 15, 1898. Serial No. 683,494. (Specimens.)

*To all whom it may concern:*

Be it known that I, WILHELM ELBERS, doctor of philosophy, a subject of the King of Prussia, German Emperor, residing at Hagen, 5 Westphalia, in the Kingdom of Prussia and Empire of Germany, have invented new and useful Improvements in the Manufacture of Gray-Indigo Coloring-Matter in Combination with Textile Fibers, of which the following is a specification.

I have invented a new article of manufacture—namely, a gray-indigo coloring-matter in combination with textile fiber—which possesses to a high degree the property of fastness against the action of light, thus rendering it possible to use fabrics of a gray shade, even in cases, such as furniture-coverings, where fastness to light is an essential. My new coloring-matter in this combination possesses the same fastness against acids and chlorid of lime and gives the same reactions as indigo-blue. It can be discharged with chromic acid and other colors printed on, so that goods with various effects on a gray 25 ground are obtained.

My invention opens up a new field of utility to the coloring-matter indigo, which can, with its assistance, be utilized for the manufacture of gray goods, whereas hitherto it 30 by itself could only be used for obtaining blue shades.

All hitherto-known processes for fixing indigo, except, of course, the sulfoacids of indigo on the different textile fibers, are based 35 upon the fact that the insoluble indigo-blue is first reduced to soluble indigo-white by means of reducing agents. Then the textile fiber is impregnated with the indigo-white in a suitable manner by dyeing or printing, and 40 then the indigo-white is on the fiber again converted into indigo-blue by oxidation, preferably by means of the oxygen of the air.

My invention consists in the production of a gray-indigo dyestuff in combination with 45 textile fiber, and I use no reduction process. The process for this production consists, substantially, in mixing finely ground or divided indigo with preferably comparatively large quantities of oils or oil derivatives, thickening 50 it with suitable substances, and then printing it on or impregnating with it the textile fiber, then subjecting the tissue to the action of steam for about one or two hours,

washing and soaping. In order to fix the color completely, the action of steam must 55 continue for a long time, but it is not absolutely necessary to use high-pressure steam, only of course the operation takes correspondingly longer when low-pressure steam is employed. Hereby is to be observed that 60 steaming at too high a pressure has an injurious effect on woolen and silk fibers, wherefore in these cases the steaming operations must be made longer and the pressure lower. The fabric thus obtained is of a good uniform 65 blue-gray color. The addition of a comparatively-large quantity of the oils as mentioned—as, for instance, olive-oil, sesame-oil, castor-oil, fat, and the like—is essential to the complete success of the process, as, 70 although the new gray coloring-matter in combination with the fiber can be obtained without it quite as fast, still the goods are not of so uniform a shade as with its addition. I have further found that the fastness or durability of the fabrics containing my new gray 75 coloring-matter in combination with the fiber can be considerably increased by subjecting the fabric printed or dyed—that is, padded with indigo—after it has been steamed and 80 freed from thickening or gum to a second steaming for a considerable time under a comparatively-high pressure. The essential point is to remove by washing and treating with malt all traces of gum or thickening from the 85 fabric before subjecting it to this second steaming operation. A much longer or frequently-repeated steaming of the unwashed fabric has far less effect than a steaming repeated after the fabric has been completely 90 deprived of gum or thickening (by washing and treating with malt) between the two steaming operations. It is also important to effect the second steaming operation at a comparatively-high pressure. This second steaming 95 operation is preferably to be used for obtaining the gray-indigo coloring-matter in combination with the cotton fiber, and it is especially important for fabrics which are required to have great fastness or permanency 100 under friction and soap—as, for instance, in “washing” fabrics for dresses.)

The following examples will serve to further illustrate the nature of my invention and the manner in which it can best be carried 105 into practical effect.

*Example 1—Production of the coloring-matter in combination with cotton by a printing process.*—The printing-color is made up of one hundred (100) parts of finely-ground indigo paste containing twenty per cent. (20%) "indigo," (including under this term refined indigo and artificial indigo of the same strength,) two hundred (200) parts of olive-oil, and seven hundred (700) parts of tragacanth gum for thickening. This coloring mixture is printed on bleached cotton fabrics, then subjected to the action of steam of 0.1 atmosphere for about three to four hours, whereby the new gray to blue-gray coloring-matter is generated in combination with the fiber. Then the gum is removed and the fabric treated with soap.

*Example 2—Production of the new gray coloring-matter in combination with cotton fiber by a padding or dyeing process.*—To obtain the gray color in combination with cotton by a dyeing or padding process, mix one hundred (100) parts of finely-ground twenty-per-cent. (20%) indigo paste, two hundred (200) parts of ricinoleate of soda, seven hundred (700) parts of tragacanth water. The fabric to be dyed is impregnated or padded with this dye with the aid of a hot flue, then subjected for about two hours to the action of steam at about 0.7 to 1.0 atmosphere pressure, whereby the new gray coloring-matter is developed on the fiber. Then the fabric is malted and soaped.

*Example 3—Production of the new gray coloring-matter in combination with wool or silk.*—Woolen or silk fabric prepared for printing in the usual way is printed upon with the following dye mixture: about nine hundred and sixty to nine hundred (960 to 900) parts of thickening material, about twenty to fifty (20 to 50) parts of indigo, and about twenty to fifty (20 to 50) parts of olive-oil. After the printing the fabric is steamed for two hours without pressure, whereby the new coloring-matter is developed. The fabric is then well washed and finished.

*Example 4—Production of the new gray coloring-matter in combination with cotton adopting a second steaming operation.*—The fabric prepared for printing in the usual way is printed on with a color mixture constituted, say, as follows: about nine hundred and sixty to nine hundred (960 to 900) parts of thickening material, about twenty to fifty (20 to 50) parts indigo paste, (containing twenty per cent. (20%) indigo,) and about twenty to fifty (20 to 50) parts of olive-oil. After the printing the fabric is steamed for about two hours at 0.1 atmosphere pressure, then washed, treated with malt, washed, and dried. It is then steamed again for about one hour and a half at, say, 0.7 to 1.0 atmosphere pressure and finished in the usual manner.

My new gray-indigo coloring-matter in combination with the fibers possesses the following characteristic properties: it can be drawn off the fabric in the same manner as indigo-

blue by heating a test portion with a solvent—as, for instance, analin, glacial acetic acid, chloroform, and the like—and also by 70 means of reducing agents—as, for instance, zinc-dust and caustic soda, hydrosulfite, and the like—and the solutions so obtained contain ordinary indigo or indigo-white. By rubbing the fabrics containing my new gray 75 coloring-matter combined with the fiber with a cloth the place rubbed shows a blue-indigo shade, not only on cotton, but also on wool and silk. When the gray indigo is prepared with a solution of grape-sugar and then printed 80 with thickened caustic soda and shortly steamed, it is also converted into indigo-blue on the printed places, the gray coloring-matter being apparently reconverted in ordinary blue indigo. By printing potassium chromate 85 on the gray indigo and drawing the tissue through a sulfuric and oxalic acid bath then the gray indigo on the printed places becomes oxidized and destroyed in a manner similar to indigo-blue, the gray color becoming 90 discharged to white. When suitable yellow, red, or green colors and albumen are added to the potassium chromate, colored effects can be produced on the gray ground in the same way as hereto on an indigo-blue ground. 95

Save in combination with the fiber as herein described no means are known for the production of the new gray-indigo coloring-matter.

Now what I claim is—

1. As a new article of manufacture a gray-colored fabric composed of textile fibrous material and indigo and having a high degree of fastness to light, acids and chloride of lime (bleaching powder) and which can be removed from the fiber by solvents or reducing mixtures as specified, yielding solutions of indigo or indigo-white and which by rubbing with a cloth or steaming with grape-sugar and caustic soda assumes an indigo-blue color and which can be oxidized and destroyed by acid 100 oxidation, all substantially as described.

2. A process for the production of gray-indigo coloring-matter in combination with the fiber consisting in printing a paste of finely-divided indigo, a suitable thickening and a 105 quantity of oil on the fiber and steaming and working up all substantially as hereinbefore described.

3. A process for the production of gray-indigo coloring-matters in combination with the 110 fiber consisting in printing a paste of finely-divided indigo, a suitable thickening and a quantity of oil on the fiber and steaming, then freeing from thickening by washing and treating with malt, drying and subjecting to a second steaming operation all substantially as 115 hereinbefore described.

In testimony whereof I have hereunto set my hand in the presence of two subscribing witnesses.

WILHELM ELBERS.

Witnesses:

R. E. JAHN,  
OTTO KÖNIG.